

# United States Patent Office

3,556,799

Patented Jan. 19, 1971

1

**3,556,799**  
**LIGHT-SENSITIVE SILVER HALIDE COLOR**  
**PHOTOGRAPHIC MATERIAL CONTAINING**  
**A MONO-PYRAZOLONE COUPLER AND A**  
**BIS-PYRAZOLONE COMPOUND**

Toshihiko Yamamoto, Mitsuto Fujiwara, Tamotsu Kojima, and Kenro Sakamoto, Tokyo, Japan, assignors to Konishiroku Photo Industry Co., Ltd., Tokyo, Japan  
 No Drawing. Filed Sept. 11, 1967, Ser. No. 666,936  
 Claims priority, application Japan, Sept. 19, 1966,

41/61,483

Int. Cl. G03c 1/40

U.S. Cl. 96—100

3 Claims

## ABSTRACT OF THE DISCLOSURE

Color staining of conventional mono-pyrazolone magenta couplers in photographic materials is prevented by using, together with the mono-pyrazolone, a bis-pyrazolone in an amount of 1-50% by weight based on the mono-pyrazolone. The bis-pyrazolone has the formula:



wherein R is alkyl, aryl or substituted aryl and R' is hydrogen, alkyl, aryl, substituted aryl or a heterocyclic radical with the proviso that at least one of R and R' contains an aliphatic hydrocarbon radical of 12-20 carbon atoms.

This invention relates to a light-sensitive photographic material useful in color photography. Particularly, the invention is concerned with a light-sensitive, color photographic material to yield a magenta color image, which comprises a magenta coupler of the mono-pyrazolone

2

type, wherein a bis-pyrazolone compound of the general formula



wherein R is alkyl, non-substituted or substituted aryl, R' is hydrogen, alkyl, non-substituted or substituted aryl, or a heterocyclic radical with the proviso that at least one of R and R' should contain an aliphatic hydrocarbon radical having 12 to 20 carbon atoms is incorporated in the photographic material. It is a principal object of the present invention to provide a light-sensitive color photographic material which is free from color staining (magenta fog) during color development.

As is well known, there are many magenta couplers which are capable of forming of magenta color image in a light-sensitive, color photographic material. Among these, a magenta coupler of the mono-pyrazolone type can give a stable color image with good tone quality at high speed. However, a photographic material in which the magenta coupler alone is incorporated is disadvantageous because it suffers from color staining during storage or development. Particularly, a magenta coupler of the mono-pyrazolone type, the pyrazolone ring of which is substituted at the 3-position with a long chain alkyl group, is very likely to cause color staining. Heretofore it was therefore necessary to use a magenta coupler of the mono-pyrazolone type in combination with an antifogging (stabilizer) such as 2,4-di-tert. butyl hydroquinone, etc. However, the use of such a stabilizer invariably causes a serious decrease in the sensitivity of high speed photographic emulsion.

In accordance with the present invention there is provided a light-sensitive, color photographic material which contains a magenta coupler of the mono-pyrazolone type which is completely prevented from color staining while retaining all the advantages inherent in said magenta coupler.

Any compound of the pyrazolone type which is heretofore known may be used as the magenta coupler of the present invention. Typically useful compounds are the following:





1-(4-sulfo-phenyl)-3-tetradecylamino-5-pyrazolone.



1-(3-carboxy-phenyl)-3-(4-palmitoylamido-phenylamino)-5-pyrazolone.



1-phenyl-3-(3-sulfopalmitoylamido-benzamido)-5-pyrazolone.



$\text{C}_{18}\text{H}_{37}$  1-(4-carboxy-phenyl)-3-(4- $\beta$ -octadecylsuccinmonoamido-phenyl)-5-pyrazolone.



1-(4-sulfo-phenyl)-3-stearoylamido-5-pyrazolone.



1-[6-sulfo-benzothiazoyl-(2)]-3-heptadecyl-5-pyrazolone.



1-heptadecyl-3-(4-carboxyl-phenyl)-5-pyrazolone.

It should be noted that the above-indicated mono-pyrazolone compounds are merely illustrative and are not

to be construed as limiting the scope of the invention thereto.

In accordance with the present invention, a magenta

coupler of the pyrazolone type as referred to above is used together with a bis-pyrazolone compound of the

above-indicated formula which typically may be the following:





These bis-pyrazolone compounds when used above (i.e. without addition of a magenta coupler of the mono-pyrazolone type) will give a clear stable color image which may be increased in maximum color density because of their bimolecular coupling reaction. However, when they are used in a high speed, color photographic emulsion, they are inferior in coupling activity and occasionally fail to give the desired photographic speed.

Such drawback of the bis-pyrazolone compounds as mentioned above can be avoided by jointly using the known mono-pyrazolone type magenta coupler in a light-sensitive, color photographic material. In accordance with the invention there is thus provided a light-sensitive, color photographic material which can give a stable color image with good tone quality at desired high speed.

The required amount of the bis-pyrazolone compound to be added may vary depending on the type of magenta coupler of the mono-pyrazolone type and further on the type of bis-pyrazolone compound used but it usually will be within the range of 1-50% by weight based on the weight of the magenta coupler. Incorporation of the specific compound of the bis-pyrazolone type into a photographic material of the present invention can be made in the manner heretofore known per se in the art. For example, it is possible to add the compound to a light-sensitive, color photographic emulsion containing a magenta coupler of the mono-pyrazolone type at any time just before, during or after the second ripening of the said emulsion. Addition of the bis-pyrazolone compound as a stabilizer for the magenta coupler is most preferably made at the stage after the second ripening. Alternatively, the bis-pyrazolone compound may be added to a starting material for the preparation of the emulsion, for example gelatine. It is desirable to add the bis-pyrazolone compound in solution dissolved in a suitable solvent, e.g. water, dilute alkali, methanol, ethanol, etc., if the addition is made to an emulsion.

Use of the bis-pyrazolone compound as a stabilizer does not adversely influence the sensitivity of the color photographic emulsion concerned. The photographic emulsion containing the said bis-pyrazolone compound can be sensitized with a gold, sulfur or other chemical or optical sensitizer.

As is well known to those skilled in the art, the term, "a light-sensitive, color photographic emulsion" or the like expression used herein is to be understood to mean any conventionally known light-sensitive, color photographic emulsion which contains a magenta coupler of the mono-pyrazolone type. A suitable color photographic emulsion will be available with reference to "Kagaku-Shashin-Binran" (Manual of Photographic Science), vol. I, pp. 455-460 (Maruzen Co., Tokyo, Japan).

25 The emulsion to which the bis-pyrazolone compound has been added can be applied to a suitable support in the manner heretofore known per se in the art, e.g. coating or pouring. Suitable supports include films, papers and glass plates. Particularly suitable are films of the types, such as cellulose esters, e.g. cellulose triacetate; polyesters obtained by the polycondensation of phthalic, isophthalic or terephthalic acid with a dihydric alcohol, e.g. polyethylene terephthalate, poly[cyclohexane-1,4-dimethyloxy]terephthalate, etc.; and polycarbonates including those obtained by the polycondensation of bisphenol A 30 with carbonic acid.

35 The present invention will now be explained in detail in conjunction with the following examples.

#### EXAMPLE 1

40 8 g. of the magenta coupler of the above-indicated Formula 1 and 2 g. of the bis-pyrazolone compound of the above-indicated Formula IX are dissolved in 35 ml. of 1 N sodium hydroxide. The resulting solution is diluted with 400 ml. of water and then added to 1 kg. of a green 45 light-sensitive, high speed photographic gelatino-silver iodobromide emulsion. Then, the emulsion is adjusted to pH 7.0 and coated on a cellulose acetate film support and dried. The thus obtained film is exposed to green light and treated at 20° C. for 10 minutes with a color developer having the following formulation:

|                                        | G.   |
|----------------------------------------|------|
| N,N-diethyl-p-phenylenediamine sulfate | 2.0  |
| Sodium sulfite (anhydrous)             | 2.0  |
| Sodium carbonate monohydrate           | 82.0 |
| 55 Potassium bromide                   | 2.0  |
| Water to make up 1000 ml.              |      |

The treated film is then treated by stopping and fixing in the usual manner. After rinsing for 10-20 minutes, this 60 film was treated for 5 minutes with a bleaching solution of the following formulation:

|                           | G.  |
|---------------------------|-----|
| Potassium ferricyanide    | 100 |
| Potassium bromide         | 50  |
| Water to make up 1000 ml. |     |

The bleached film is treated by rinsing, fixing and rinsing in the usual manner. After drying, the film is subjected to sensitometry.

70 On the other hand, two control samples are prepared in substantially the same manner as above but using in the control sample (1) 10 g. of the magenta coupler of the above-indicated Formula 1 alone and in control sample (2) 10 g. of the same magenta coupler and 500 mg. of 2,4-di-tert. butyl hydroquinone, instead of the magenta coupler and bis-pyrazolone compound used in

Example 1. These control samples also are subjected to sensitometric tests.

The test results are set forth in Table 1.

TABLE 1

|                          | Photographic speed | Fog  |
|--------------------------|--------------------|------|
| Sample of Example 1..... | 97                 | 0.08 |
| Control sample (1).....  | 100                | 0.17 |
| Control sample (2).....  | 70                 | 0.13 |

In the above and also in Tables 2 and 3 which appear later, photographic speed values are expressed as relative values based on the speed of the control sample (1) which is rated as 100.

Separately, two sets of the above three film samples are stored under the following condition:

Condition A.—For seven days at a temperature of 50° C. under a relative humidity of 20%.

Condition B.—For five days at a temperature of 55° C. under a relative humidity of 80%.

After the specified storage, each set of the films are treated by color development in the same manner as before and then tested by sensitometry. The results are set forth in Table 2.

TABLE 2

|                         | Condition A         |      | Condition B         |      |
|-------------------------|---------------------|------|---------------------|------|
|                         | Photo-graphic speed | Fog  | Photo-graphic speed | Fog  |
| Sample of Example 1.... | 100                 | 0.18 | 145                 | 0.25 |
| Control sample (1)..... | 100                 | 0.38 | 100                 | 1.01 |
| Control sample (2)..... | 90                  | 0.22 | 120                 | 0.50 |

Color images obtained by using the samples of Example 1 are excellent in tone quality and stability.

### EXAMPLE 2

7 g. of the magenta coupler of the above-indicated Formula 7 and 3 g. of the bis-pyrazolone compound of the above-indicated Formula IV are dissolved in 30 ml. of 1 N sodium hydroxide. The resulting solution is diluted with 500 ml. of water and added to 1 kg. of a green light-sensitive gelatino-silver chlorobromide emulsion, which is then adjusted to pH 6.9 with citric acid and coated on a cellulose acetate film support. The resulting film is treated in the same manner as in Example 1 to obtain the results given in Table 3.

On the other hand, two control samples are prepared

by using in the control sample 3 10 g. of the magenta coupler of the Formula 7 alone and in the control sample 4 10 g. of the same magenta coupler and 500 mg. of 2,4-di-tert. butyl hydroquinone. These control samples also are tested by sensitometry.

TABLE 3

|                          | Photographic speed | Fog  |
|--------------------------|--------------------|------|
| Sample of Example 2..... | 126                | 0.02 |
| Control sample (3).....  | 100                | 0.07 |
| Control sample (4).....  | 85                 | 0.05 |

What we claim is:

1. A light-sensitive, color photographic material which comprises on a support a light-sensitive gelatino-silver halide emulsion layer containing a magenta coupler of the mono-pyrazolone type and a bis-pyrazolone compound of the formula



wherein R is alkyl, aryl or carboxyl, sulfo or amido substituted aryl radical and R' is hydrogen, alkyl, aryl, carboxyl, sulfo or amido substituted aryl or heterocyclic radical, with the proviso that at least one of said R and R' contains an aliphatic hydrocarbon radical having 12-20 carbon atoms in an amount sufficient to prevent color staining with said magenta coupler.

2. A light-sensitive, color photographic material as claimed in claim 1, wherein said photographic material is a tricolor photographic film.

3. A light-sensitive, color photographic material as claimed in claim 1, wherein said bis-pyrazolone compound is present in the amount of 1-50% by weight based on the weight of said magenta coupler.

### References Cited

#### UNITED STATES PATENTS

2,411,951 12/1946 Bauley ..... 96-100  
2,728,659 12/1955 Loria et al. ..... 96-56

45 J. TRAVIS BROWN, Primary Examiner

U.S. CL. X.R.